

## UNITED STATES PATENT OFFICE.

PORTER H. BRACE, OF PITTSBURGH, PENNSYLVANIA, ASSIGNOR TO WESTINGHOUSE ELECTRIC & MANUFACTURING COMPANY, A CORPORATION OF PENNSYLVANIA.

## PERMANENT-MAGNET STEEL.

No Drawing.

Application filed January 16, 1919. Serial No. 271,480.

My invention relates to magnetic materials and more particularly to permanent-magnet steels, and it has for its primary object the provision of a permanently magnetizable 5 steel which may be manufactured at a cost materially below that of steels of that character, heretofore known.

A further object of my invention resides in the provision of a magnetizable steel, or 10 steel alloy, which shall be superior to those heretofore known, in that it shall have less tendency to crack while hardening during its manufacture and during heat treatment.

I have found, as a result of investigating 15 the magnetic properties of steel, that the addition of cobalt and one or more of the metals of the chromium group, or vanadium to steel, produces an alloy having characteristics which make it well suited for use in 20 the manufacture of permanent magnets. While the metal or metals of the chromium group to be employed with the cobalt may, preferably, be varied to suit slightly different requirements of use, I have found 25 that, from standpoints of cost and general utility, a chromium-cobalt steel is usually to be preferred.

Although the proportions of the cobalt and of the chromium or other metal or 30 metals of the chromium group, such as molybdenum and tungsten, to be employed may likewise be varied to suit different conditions, it is preferable, from the viewpoint 35 of economy, if for no other reason, that the quantities of such metals be as small as possible. I have found that steel compositions ranging from 1% to 10% cobalt, 1% to 10% chromium, and the remainder iron and minor impurities, are particularly desirable.

40 Previous to this, tungsten steels have been the most extensively used of all steel alloys, or equivalent metals, in the manufacture of permanent magnets and, when properly hardened, such steels show, under suitable 45 tests, the following magnetic characteristics:

Maximum induction..... 16,000-17,000  
Remanent induction..... 7,300-7,600  
Coercive force..... 84-86

50 In comparison with these characteristics, I have obtained the following results from

similar tests made with chromium cobalt steels:

|                         |               |    |
|-------------------------|---------------|----|
| Maximum induction.....  | 17,000-18,000 | 55 |
| Remanent induction..... | 7,300-7,500   |    |
| Coercive force.....     | 81-86         |    |

While the quantities of both the cobalt and the chromium or other metal of the chromium group or an equivalent mixture 60 of such metals may vary, the following tables give two characteristic analyses of chromium-cobalt steels which have been found to be satisfactory.

65

|         | #1    | #2   |
|---------|-------|------|
| Cr..... | 4.75  | 3.17 |
| Co..... | 5.00  | 2.89 |
| C.....  | 0.53  | 0.77 |
| Mn..... | 0.60  | 0.78 |
| P.....  | 0.025 | 0.02 |
| S.....  | 0.018 | 0.02 |

70

The remainder Fe and minor impurities.

Through actual experience in making steel 75 alloys of the above described character, I have found that, during the hardening of the molten alloy and its subsequent heat-treatment, there is much less tendency to cracking than is the case with the tungsten 80 steels previously used. The heat treatment to which the alloy is subjected may be that heretofore ordinarily employed in the making of magnet steels, which was to heat them to a red heat and to then quench them, at 85 this temperature, in either oil or water, although it will be understood by those skilled in the art that a higher or lower temperature may be employed.

A permanent magnet may be produced by 90 subjecting a body of the hardened alloy, having suitable form and dimensions, to the influence of a magnetic field for a few moments, as, for example, by passing an electric current through an insulated wire 95 wrapped around the body to be magnetized, as is well known in the art.

Heat treatment of steels to be utilized in the making of magnets and the process of making magnets therefrom are well known 100 to metallurgists and are fully described in the literature of this art. See, for example,

page 413 of the 1908 edition of the Metallurgy of Iron and Steel by Bradley Stoughton. As it is obvious that cobalt-chromium steels are much cheaper, it will be apparent that I have provided a permanently-magnetizable steel or steel alloy possessing magnetic characteristics comparing favorably with those of the steel alloys now in use and having advantages not previously attainable.

Obviously, numerous changes in the metal or metals employed with the cobalt in forming magnetizable alloys of this character, as well as in the proportions of the alloying metals, both relative to each other and to the iron employed, may be made within suitable bounds. For example, the proportions of the cobalt may be substantially increased. An alloy containing 20% of a mixture of cobalt and chromium and the remainder iron and minor impurities has been found satisfactory. It will, therefore, be understood that, when economic conditions permit, a much higher percentage of the alloying ingredients may be employed and this is especially true of cobalt, the proportions of which may be varied within a comparatively wide range. I do not wish, therefore to, in any way, restrict my invention to the employment of any particular metals or to the use of any specific proportions but reserve the right to make all changes, both in materials employed and in proportions utilized, which may come within the scope of the appended claims.

I claim as my invention:

1. A magnetized member comprising substantially 1% to 10% cobalt, 1% to 10% of a metal of the chromium group and the remainder iron and minor impurities.
2. A magnetized member comprising substantially 1% to 10% cobalt, 1% to 10% of at least one of the following metals:

chromium, molybdenum, tungsten and vanadium and the remainder iron and minor impurities.

3. A magnetized member comprising 1% to 10% chromium, 1% to 10% cobalt and the remainder iron and minor impurities.

4. A chromium-cobalt steel for permanent magnets.

5. A magnetized member comprising from 2% to 20% of a mixture of chromium and cobalt and the remainder iron, carbon and minor impurities.

6. A magnet containing 1% to 10% cobalt and 1% to 10% of at least one metal of the chromium group.

7. A magnet containing 1% to 10% cobalt and 1% to 10% chromium.

8. As a new article of manufacture, a magnetized body of an alloy steel containing cobalt and a metal of the chromium group.

9. As a new article of manufacture, a magnetized body of an alloy steel containing cobalt and tungsten.

10. As a new article of manufacture, a permanent magnet comprising a magnetized body of an alloy steel containing a substantial percentage of cobalt substantially uniformly distributed therethrough.

11. As a new article of manufacture, a magnetized body of an alloy steel containing cobalt and chromium.

12. As a new article of manufacture, a magnetized body of an alloy steel containing cobalt and molybdenum.

13. A magnetized member comprising cobalt, at least one of the following metals; chromium, molybdenum, tungsten, and vanadium, and the remainder iron carbon and minor impurities.

In testimony whereof, I have hereunto subscribed my name this 31st day of Dec., 1918.

PORTER H. BRACE.